# EUROPEAN PATENT APPLICATION

(11) **EP 3 031 550 A1**
(43) Date of publication of application: **15.06.2016**
(21) Application number: 14197265.3
(22) Date of filing: 11.12.2014
(51) Int. Cl.: B22F 1/00, B22F 3/14, B22F 3/15, B22F 3/16

(54) **Method for producing sintered components by HIP**

(71) Applicant: Höganäs AB (publ), 263 83 Höganäs (SE)
(72) Inventor: Miedzinski, Artur, 263 83 Höganäs (SE); Flodin, Anders, 263 83 Höganäs (SE)

(57) **Abstract**

The present invention relates to a method for manufacturing metal components comprising the following steps;
a. obtaining a metal powder composition comprising a particulate lubricant and a metal powder, wherein the metal powder particles have a size of less than 75µm, and the lubricant particles have a size of less than 25µm;
b. compacting said metal powder composition in a mould to a density of at least 7.3g/cm³ to produce a green component;
c. sintering the green component at a temperature of at least 1300°C during at least 1 hr to produce a sintered component;
d. treating the sintered component without under a pressure of at least 900MPa during an elevation of the temperature to 1100°C; thereby obtaining a metal component having >99% of the theoretical density.

## Description

### SUMMARY

The present invention relates to a method for producing sintered components by hot isostatic pressing (HIP). The method is a simplified method compared to known methods, and produces components having high density, without the need for encapsulation or surface treatment.

### BACKGROUND

Powder metallurgy is mainly a producing technique where compacted powder is bound together by sintering. The metal powders and the components normally have a rather basic composition. In some cases, other alloying elements are added to provide better mechanical properties. The technique is suitable for producing components, such as gears. Other benefits for powder metallurgy are net Shape, high volume production and low energy consumption.

Pores are a common problem in metal components, even after sintering. When powder metals, PM, are used for the manufacture of metal components, such as gears, these may contain approximately 5-10% pores. The properties of the metal components deteriorate with the amount of pores. By eliminating pores properties like hardness, density, strength, fatigue life, and ductility are improved.

The amount of pores may be avoided with a process called hot isostatic pressing, HIP. When powder is pressed in a HIP-machine, most of the pores are removed, which gives a high density and a high fatigue for a material. High density usually gives the material high strength.

The HIP method involves the following steps: The powder mixture is placed in a container which is subjected to raised temperature and high pressure. The container may be fabricated by any material that is deformable at the consolidation temperature, and glass, steel, or stainless steel is commonly used, depending on the maximum temperature. The isostatic pressure is applied from all sides of the component and through deformation this produces a component without pores.

During the HIP-process diffusion bonds are created between similar and dissimilar elements. These bonds results in a densification of the material and makes it possible to produce a component without pores. Components without pores have improved mechanical properties such as high strain and ductility, compared with components with higher amount of pores. It has been shown that the HIP-process can remove residual stresses and stabilize the component after sintering.

Fully dense PM-gears can be produced through HIP process in a stainless steel container. This method however is too expensive to be commercially viable.

One variant of the above method is to use previously sintered components. This has the advantage of not requiring a container, but to date, it has not been possible to produce very high density components.

There is still a need for technology to produce high density components.

### SUMMARY OF THE INVENTION

The present invention provides a metal powder composition and a method for hot isostatic pressing without the need of a container. The method is a simplified version of the traditional HIP-method and is capable of producing components with more than 99% of the theoretical density.

### DETAILED DESCRIPTION OF THE INVENTION

The invention is based on the realization that a specific type of additive, namely a lubricant, can be used to enable high density components by container-free hot isostatic pressing. The lubricant is preferably of a small size, e.g smaller than 25µm, or smaller than 12µm, or preferably smaller than 5µm, or most preferably between 3 and 5µm. The lubricant may be amide wax or zinc stearate. Preferably, the lubricant is zinc stearate.

The lubricant is mixed with an atomized metal powder, preferably of a size smaller than 75µm, preferably smaller than 63µm. The powders may be e.g. Astaloy 85Mo, Distaloy AQ, ASC300(available from Höganäs AB, Höganäs, Sweden). A common way of obtaining a powder with particles smaller than a certain size is by way of sieving.

The metal powder composition is placed in a mould and compacted at a pressure of 800-1000MPa, to a density of at least 7.3g/cm³, or preferably at least 7.4g/cm³, producing a green component.

The compacted component is removed from the mould and sintered in an atmosphere of 90/10 N₂/H₂, at a temperature between 1300°C and 1350°C. The sintering takes place during a time of about 0.5hr-2hrs.

The sintered component is then subjected to hot isostatic pressure; the component is placed in a pressure chamber, pressure is raised to at least 1000MPa and the temperature is raised to at least 1000°C This HIP-step takes place during a time of at least 0.5hrs, or preferably at least 1 h. The hot isostatic pressure step is carried out without encapsulating the component in a container.

The hot isostatic pressure treatment may be performed directly following the sintering, in the same furnace. In this case, it is a matter of holding the component at an elevated pressure and temperature as described for the above mentioned HIP-stage.

Following the above HIP-treatment, the component is removed from the pressure chamber. Components treated as above have a density of >99% of the theoretical density.

### EXAMPLES

### Example 1

Metal powder compositions were prepared according to Table 1. Metal powders were sieved to remove particles larger than 63µm. Graphite and lubricant was added to all samples. Graphite amount of 0.2 wt-% and the amount of lubricant is 0.6 wt-%. The lubricant mixture Zinc-stearate has a mean particle size of approximately 3-5µm.

**Table 1**

| Sample | Powder name | Alloying element (wt-%) | Fe | Lubricant |
|---|---|---|---|---|
| 1 | Astaloy 85Mo | 0.85 Mo | Balance | Zn-stearate |
| 2 | Distaloy AQ | 0.5 Ni, 0.5 Mo | Balance | Zn-stearate |
| 3 | ACS 300 | | Balance | Zn-stearate |

### Example 2

The metal powder compositions according to Table 1 were used to press gears according to Table 2.

**Table 2**

| | |
|---|---|
| Number of teeth | z=18 |
| Module | mₙ=1.5875 mm |
| Pressure angle | α=20° |
| Face width | b=10mm |
| Centre distance | a=35.72 mm |

### Example 3

The gears manufactured in Example 2 were compacted at 800-1000MPa to achieve maximum density. One batch was sintered at 1120°C, 60min, N₂-95%, H₂-5%; a second batch sintered at 1250°C, 60min, 95%N₂-5% H₂; and a third batch sintered at 1300°C, 120min, 95%N₂-5% H₂. The densities where measured according to Archimedes principle, and given in Table 3.

### Example 4

The sintered gears from Example 3 were treated under similar conditions, at a temperature of 1100°C and a pressure of 1000MPa, during 2hrs. Table 3 shows the density of the gears before and after high isostatic pressure treatment.

The experiments have shown that it is possible to press, sinter and HIP PM components, without using a container, to a density of more than 99% of the theoretical density. It is also shown that the alloying elements are not very relevant for the densification using HIP. During the experiments, all materials densified to high density.

## Claims

1. Method for manufacturing metal components comprising the following steps;
a. obtaining a metal powder composition comprising a particulate lubricant and a metal powder, wherein the metal powder particles have a size of less than 75µm, and the lubricant particles have a size of less than 25µm;
b. compacting said metal powder composition in a mould to a density of at least 7.3g/cm³ to produce a green component;
c. sintering the green component at a temperature of at least 1300°C during at least 1 hr to produce a sintered component;
d. treating the sintered component without under a pressure of at least 900MPa during an elevation of the temperature to 1100°C; thereby obtaining a metal component having >99% of the theoretical density.
